

Feb. 27, 1934.

G. TAYLOR

1,949,338

## PROCESS OF MAKING HAIR CLOTH

Filed May 9, 1931



Inventor:  
George Taylor  
by his Attorneys  
Harrison & Harrison

## UNITED STATES PATENT OFFICE

1,949,338

## PROCESS OF MAKING HAIR CLOTH

George Taylor, Philadelphia, Pa.

Application May 9, 1931. Serial No. 536,283

8 Claims. (Cl. 28—1)

This invention relates to the manufacture of hair cloth. In weaving hair cloth, natural hair, taken from the tail of a horse, is commonly employed as the weft and the width of the fabric is limited to the maximum length of the available hair, it being noted that each strand of hair extends the full width of the fabric, from selavage to selavage thereof. Natural horse hair does not exceed 36 inches in length and the necessary allowance for variations in the length of the strands and allowance for the grippers of the shuttle which draws the hairs one at a time through the open warp shed, reduces the actual width of the finished fabric considerably below the length of the hair; for example, when using 36 inch hair the width of the finished fabric is approximately 30 inches. In most cases, however, 36 inch hair is not obtainable and consequently the width of the fabric runs from 20 to 24 inches.

The object of this invention is to produce a hair cloth fabric having a width substantially greater than the maximum length of natural horse hair obtainable; for example, hair cloth fabric having a width of 54 inches more or less, which makes the fabric adaptable for use in the upholstering of large pieces of overstuffed furniture, etc., where the use of hair cloth is extremely desirable from the point of service, appearance, etc. Prior to this invention the use of hair cloth as the upholstery for such large pieces of furniture was impossible, due to the relatively narrow width of the hair cloth obtainable.

Hair cloth has been commonly used in the past in upholstering smaller pieces of furniture and in certain automobiles where the narrower fabric could be used to advantage.

Natural horse hair is not uniform in diameter throughout its entire length, the butt end of the hair being slightly larger in diameter than the outer end of the hair.

Another object of the invention is to provide hair which will be uniform throughout its entire length whereby the entire area of the finished fabric will have a uniform appearance.

These objects are obtained by using a synthetic horse hair, in the present instance composed of a cellulose filament, having a diameter substantially the same as natural horse hair, and being of the general character and composition as what is generally known on the market as "rayon."

The cellulose filament employed in the present instance is of a considerably heavier gage than the cellulose threads commonly used in the manufacture of knitted or woven artificial silk fabrics and is therefore of a relatively stiffer nature, which

prevents of its being wound on bobbins or formed into cops, such as are employed in shuttles used in the weaving of textile fabrics in general. If wound onto a bobbin or into a cop the tendency of the heavier gage cellulose filament is to unwind in a manner similar to a coil of fine spring wire and furthermore, in being so wound, the cellulose filament assumes the nature of a series of convolutions, which destroys its value as a weft in the manufacture of hair cloth wherein the weft must be straight and relatively stiff.

A further object of the invention therefore resides in the preparation of the cellulose filament to eliminate all kinks or undulations from the filament, in order that it will be straight and adaptable for use in an ordinary hair cloth loom to be handled by the hair-selecting mechanism of the loom, in the same manner as natural horse hair is handled at the present time. For this purpose, I employ a loom similar to that shown and described in my prior United States Letters Patent No. 805,806, dated April 16, 1907. The only modification made in the loom disclosed in this patent is that the lay, breast beam, and similar elements extending transversely of the loom are increased in length, in order to accommodate the wider fabric, no modification of the operating elements of the loom being necessary.

The preparation of the cellulose filament will be more fully described hereinafter, reference being had to the accompanying drawing, of which:

Fig. 1 is a diagrammatic face view of a small piece of fabric made in accordance with the principles of this invention;

Fig. 2 is a diagrammatic warp-wise section taken on the line 2—2, Fig. 1;

Fig. 3 is a diagrammatic view of a skein of cellulose filament as it is purchased on the open market;

Fig. 4 is an elevation of a frame showing the skein of cellulose filament thereon, in the first step of the course of preparation of the filament for weaving purposes;

Fig. 5 is a view similar to Fig. 4 but showing the skein of filament in a subsequent stage of the preparation;

Figs. 6 to 11 inclusive show other subsequent steps in preparing the filament for the loom;

Fig. 12 diagrammatically illustrates the filament encased in a protective covering ready for placement in the loom to weave the fabric; and

Fig. 13 is a transverse section taken on the line 13—13, Fig. 12.

Referring to Fig. 3, a skein cellulose filament is generally illustrated at A, said skein being com-

posed usually of one continuous filament  $a$  loosely coiled in the manner illustrated. Such filament, as it is purchased on the market, has an inherent stiffness or spring-like nature and is of a more or less wavy formation, the undulations being relatively long as illustrated at  $a^1$ , Fig. 3.

The filament as purchased on the open market is of a neutral color and before it is woven or otherwise formed into a finished fabric the filament must undergo a dyeing process. When the skein of filament is dampened or wet, as in dyeing, the convolutions of the filament  $a$  immediately form into a series of relatively small undulations or kinks as illustrated at  $a^2$  in Fig. 4.

In order to remove these and all other undulations and kinks from the dampened filament, and to produce in the filament a straight condition, similar to horse hair, the apparatus shown in Figs. 4 and 5 is employed.

For the purpose of illustrating this straightening process the frame, illustrated in Figs. 4 and 5, may be described as comprising an upper rail 1 rigidly supported in any suitable manner, such for example as by vertically extending posts 2, 2, and a lower rail 3 which is adjustable vertically with respect to the upper rail 1 as and for the purpose hereinafter described. Obviously the rails 1 and 3 may be disposed in a common horizontal plane if desired.

On the rail 1 is a skein support, which in the present instance comprises a laterally extending hook, pin or peg 4, and on the lower rail 3 is a similar hook, pin or peg 5. The moistened skein A is placed on the upper support 4 and around the lower support 5 in the manner illustrated in Fig. 4. The lower rail 3 is then dropped of its own weight or force downwardly, if desired, to tighten the skein A between the supports 4 and 5 against the inherent tendency of the filament to form into the small undulations  $a^2$ .

Pins 6, 6 or other corresponding means is provided for securing the lower rail 3 in a relatively fixed position with respect to the upper rail 1 in the present instance. The lower rail 3 is shown as being provided with openings 7 for the reception of the pins 6 and the uprights 2, 2 are likewise provided with openings 8, 8 into which the pins 6, 6 extend for the purpose of preventing vertical movement of the support 5 as the filaments  $a$  of the skein A shrink in drying. As the filament  $a$  dries it shrinks considerably, but due to the relatively fixed positioning of the supports 4 and 5 the shrinking of the filaments  $a$  places the skein A under extremely high tension. The skein A is permitted to stand until thoroughly dried and due to the high tension produced by the shrinking of the filaments all semblance of undulations or kinks is removed from the filament, consequently the filament assumes and maintains a straight condition thereafter, such as illustrated at  $a^3$  in Fig. 5.

After the skein is thoroughly dried, the pins 6 are released, permitting the support 5 to be moved toward and support 4 in order that the skein may be removed from the supports 4 and 5, the skein then having the appearance illustrated in Fig. 6 comprising groups of straight parallel filaments  $a^3$ ,  $a^3$  connected by curved portions  $a^4$ ,  $a^4$  at the opposite ends of the dried skein. The parallel groups of straight filaments  $a^3$ ,  $a^3$  are then bound together as illustrated at  $b$ ,  $b$  in Fig. 7, after which the curved ends  $a^4$ ,  $a^4$  of the skein are severed outside the bindings  $b$ ,  $b$  as illustrated in Fig. 8; thus the skein A is con-

verted into a bundle of individual parallel strands as illustrated at B in Fig. 8.

In order to insure the parallel relationship of the individual strands of the bundle B the said bundle is then put through a combing operation, the comb being diagrammatically illustrated at 10 in Fig. 9, one of the end bindings  $b$  being removed and the opposite end remaining bound as illustrated in Fig. 9, after which a relative longitudinal movement of the comb with respect to the bundle of filaments B is effected toward the unbound end of the bundle. After thorough combing of this one end the binding  $b$  is then applied to the combed end and the binding  $b$  at the opposite end of the bundle is then removed and the combing operation repeated. Such combing of the bundle of filaments B insures parallel relationship of the individual filaments or strands and eliminates any twisting of the individual strands which may have occurred during the previous steps in the process. The combing also removes any strands that may contain knots such as have been made in the filament  $a$  during the winding or reeling thereof into the skein A.

After the bundle of filaments B has been thoroughly combed and the end bindings  $b$ ,  $b$  have been applied in the manner illustrated in Fig. 10 intermediate bindings  $b^1$ ,  $b^1$  are applied in the manner and at the places illustrated in Fig. 10, to prevent any subsequent twisting or tangling of the strands in the bundle.

Due to the severing of the curved portions  $a^4$ ,  $a^4$  of the bundle B, as illustrated in Fig. 8, the filaments comprising the bundle B are not of uniform length and the ends beyond the bindings  $b$ ,  $b$  respectively are somewhat curved, and in order to remove the curved ends and to make all the strands in the bundle the same length the irregular ends of the bundle are cut off in the manner illustrated at  $a^5$  in Fig. 11.

The bundle B is then placed in a suitable casing, such as illustrated in Fig. 12. This covering may be of a tubular nature, or it may be in the form of a sheet in which the bundle is laid and rolled as illustrated in Figs. 12 and 13, with the opposite edges of the sheet overlapping to form a substantially tubular cover around the bundle B, suitable straps or other bindings  $c$  being provided to secure the casing in position.

The binding  $b$  adjacent the end of the bundle which is left protruding from the open end of the casing C is then removed. The other bindings  $b^1$  and the binding  $b$  at the opposite end of the bundle B may be permitted to remain around the bundle, if desired, but preferably these bindings are removed before the bundle is enclosed within the casing C. In any event the casing C provides a protective covering for the bundle, preventing any tangling or breaking of the filaments in the handling of the bundle while it is being placed in the hair trough of the loom, such as illustrated in the patent above noted.

The bundle of filaments in the condition shown in Fig. 12 is then ready for placement in the loom, wherein the individual strands are picked up one at a time by the shuttle mechanism of the loom, alternately from opposite sides of the loom and drawn through the open warp shed to form the wefts  $x$  of the fabric illustrated in Fig. 1, these wefts  $x$  being tied in, in the usual manner common in hair cloth looms, by the chain warps  $y$ ,  $y$ , to complete the fabric on the loom. Obviously the bundles in the troughs at the opposite sides of the loom may be of different colors, whereby a two-tone or multi-colored fabric is produced.

In Figs. 1 and 2, a common over-one-under-one weave is shown, merely for the purpose of illustration, but it will be understood that any desired weave may be employed such as are common in natural-hair cloth, for the production of patterns or other design effects in the fabric to make it suitable for upholstery purposes, the plain weave fabrics, such as illustrated in Figs. 1 and 2, being commonly employed as a stiffening agent 10 in the making of men's and women's coats and other wearing apparel where a foundation is provided.

In order to make the fabric more suitable for upholstery and similar purposes, I provide on the 15 one face of the fabric a suitable backing  $z$ . This backing may be of any desired nature and of any desired color to produce a suitable background for the superposed design. Preferably this backing fabric is of a water-proof nature. The 20 backing  $z$  is preferably secured to the one face of the hair cloth fabric by the use of any suitable adhesive such as a flexible cement or glue which may be purchased on the open market.

Cellulose filaments usually have a high lustre 25 and it has been observed that the shrinking under restriction as above noted tends to accentuate the lustre and cause it to take on an appearance which so closely resembles the appearance of natural horse hair that it is practically impossible 30 to differentiate between the two without resorting to scientific analysis.

From the above, it will be quite obvious that the wefts  $x$  may be made to any length desired and the width of the fabric will be limited only by the 35 width of the loom on which the fabric is to be woven.

I claim:

1. The process for preparing cellulose filament for use in a fabric of the hair cloth type, comprising dampening of the filament in skein, stretching the skein between a pair of relatively spaced supports until dry, to form and set the skein into groups of straight substantially parallel strands interconnected by end portions engaged by said 45 supports, and removing the said end portions, to provide separate rectilinear strands.

2. The process for preparing cellulose filament for use in a fabric of the hair cloth type, comprising dampening the filament in skein, stretching the 50 dampened skein between a pair of relatively spaced supports until dry, to form the skein into groups of straight substantially parallel strands, binding the dried elongated skein adjacent the opposite ends thereof, and severing the 55 connections between the parallel groups to form the skein into a bundle of individual strands.

3. The process for preparing cellulose filament for use in a fabric of the hair cloth type, comprising dampening the filament in skein, stretching the 60 dampened skein between a pair of relatively spaced supports until dry, to form the skein into groups of straight substantially parallel strands, binding the dried elongated skein adjacent the opposite ends thereof, severing the connections 65 between the parallel groups to form the skein into a bundle of individual strands, releasing the binding at one end of the bundle, and combing the bundle toward its opposite end to eliminate twisting of the individual strands.

4. The process for preparing cellulose filament for use in a fabric of the hair cloth type, comprising dampening the filament in skein, stretching the 70 dampened skein between a pair of relatively spaced supports until dry, to form the skein into groups of straight substantially parallel strands, binding the dried elongated skein adjacent the opposite ends thereof, severing the connections between the parallel groups to form the skein into a bundle of individual strands, releasing the binding at one end of the bundle, and combing the bundle toward its opposite end to eliminate twisting of the individual strands.

5. The process for preparing cellulose filament

for use in a fabric of the hair cloth type, comprising dampening the filament in skein, stretching the dampened skein between a pair of relatively spaced supports until dry, to form the skein into groups of straight substantially parallel strands, binding the dried elongated skein adjacent the opposite ends thereof, severing the connections between the parallel groups to form the skein into a bundle of individual strands, releasing the binding at one end of the bundle, 80 combing the bundle toward its opposite end to eliminate twisting of the individual strands, re-binding the one end, releasing the binding at the opposite end, and repeating the combing operation.

6. The process for preparing cellulose filament for use in a fabric of the hair cloth type, comprising dampening the filament in skein, stretching the dampened skein between a pair of relatively spaced supports until dry, to form the skein into groups of straight substantially parallel strands, binding the dried elongated skein adjacent the opposite ends thereof, severing the connections between the parallel groups to form the skein into a bundle of individual strands, releasing the binding at one end of the bundle, 85 combing the bundle toward its opposite end to eliminate twisting of the individual strands, re-binding the one end, releasing the binding at the opposite end, repeating the combing operation, 90 and subsequently encasing the combed bundle to prevent entangling of the combed strands during subsequent handlings of the bundle.

7. The process for preparing cellulose filament for use in a fabric of the hair cloth type, comprising dampening the filament in skein, stretching the dampened skein between a pair of relatively spaced supports until dry, to form the skein into groups of straight substantially parallel strands, binding the dried elongated skein adjacent the opposite ends thereof, severing the connections between the parallel groups to form the skein into a bundle of individual strands, releasing the binding at one end of the bundle, 100 combing the bundle toward its opposite end to eliminate twisting of the individual strands, re-binding the one end, releasing the binding at the opposite end, repeating the combing operation, 105 and subsequently encasing the combed bundle to prevent entangling of the combed strands during subsequent handlings of the bundle.

8. The process for preparing cellulose filament for use in a fabric of the hair cloth type, comprising dampening the filament in skein, stretching the dampened skein between a pair of relatively spaced supports until dry, to form the skein into groups of straight substantially parallel strands, binding the dried elongated skein adjacent the opposite ends thereof, severing the connections between the parallel groups to form the skein into a bundle of individual strands, releasing the binding at one end of the bundle, 115 combing the bundle toward its opposite end to eliminate twisting of the individual strands, re-binding the one end, releasing the binding at the opposite end, repeating the combing operation, 120 and subsequently encasing the combed bundle to prevent entangling of the combed strands during subsequent handlings of the bundle.

9. The process for preparing cellulose filament for use in a fabric of the hair cloth type, comprising dampening the filament in skein, stretching the dampened skein between a pair of relatively spaced supports until dry, to form the skein into groups of straight substantially parallel strands, binding the dried elongated skein 125 adjacent the opposite ends thereof, severing the connections between the parallel groups to form the skein into a bundle of individual strands, releasing the binding at one end of the bundle, combing the bundle toward its opposite end to eliminate twisting of the individual strands, re-binding the one end, releasing the binding at the opposite end, repeating the combing operation, 130 and subsequently encasing the combed bundle to prevent entangling of the combed strands during subsequent handlings of the bundle.

10. The process for preparing cellulose filament for use in a fabric of the hair cloth type, comprising dampening the filament in skein, stretching the dampened skein between a pair of relatively spaced supports until dry, to form the skein into groups of straight substantially parallel strands, binding the dried elongated skein 135 adjacent the opposite ends thereof, severing the connections between the parallel groups to form the skein into a bundle of individual strands, releasing the binding at one end of the bundle, combing the bundle toward its opposite end to eliminate twisting of the individual strands, re-binding the one end, releasing the binding at the opposite end, repeating the combing operation, 140 and subsequently encasing the combed bundle to prevent entangling of the combed strands during subsequent handlings of the bundle.

adjacent the opposite ends thereof, severing the connections between the parallel groups to form the skein into a bundle of individual strands, releasing the binding at one end of the bundle, 5 combing the bundle toward its opposite end to eliminate twisting of the individual strands, re-binding the one end, releasing the binding at the opposite end, repeating the combing operation, rebinding the last said end of the bundle, binding 10 the combed bundle intermediate said end

bindings to prevent relative movement between the strands, cutting the ends of the strands protruding beyond the bindings to produce strands of uniform length, removing the bindings from the bundle to free the strands to permit the strands to be picked from the bundle individually, and encasing the bundle to prevent entanglement of the strands during subsequent handlings of the bundle.

GEORGE TAYLOR. 85

80

15

90

20

95

25

100

30

105

35

110

40

115

45

120

50

125

55

130

60

135

65

140

70

145

75

150